

## UNITED STATES PATENT OFFICE

2,411,429

## TREATMENT OF CELLULOSEC TEXTILE MATERIALS

Horace James Hegan, Coventry, and Edwin Holroyd Sharples, Kenilworth, England, assignors to Courtaulds Limited, London, England, a British company

No Drawing. Application November 6, 1944, Serial No. 562,264. In Great Britain January 12, 1944

4 Claims. (Cl. 57—157)

1

This invention relates to treating cellulosic textile materials in order to obtain level dyeings when these materials are knitted into hosiery or woven into fabrics.

It is well known to subject cellulosic yarn or thread to a twisting operation and subsequently to set the twist by treatment with steam. When cellulosic yarns are subjected to steaming, there is a lowering of the affinity of the yarn for dye-stuffs, which lowering is dependent upon the temperature and time of the steaming and the degree of wetness of the yarn. When steaming the yarn on bobbins, there is a tendency for the outer layers of yarn to be more heavily steamed than the inner layers and also there is a possibility of drops of condensed water falling on the yarn so that there is a considerable tendency in the steaming process for variations in dyeing affinity to be produced throughout the bobbin and on making this unevenly steamed yarn into hosiery and subsequently dyeing, the material exhibits marked differences in shade.

The object of the present invention is to obtain a yarn which will be stabilised towards the steam treatment so that any differences occurring during the steaming process will not appreciably affect the dyeing affinity of the yarn, and therefore the evenness in shade of the knitted or woven material.

According to the present invention, cellulosic yarn or thread is treated in hot water at temperatures above 100° centigrade, and then dried and twisted and the twist is set by a steaming operation. The pretreatment in hot water stabilises the yarn so that any differences in the steaming operation do not deleteriously affect the dyeing affinity. The treated yarn is knitted or woven into fabric which on subsequent dyeing gives level shades.

The conditions of time and temperature used in carrying out this invention are interdependent, a higher temperature giving a desired result in a shorter time. It is sometimes preferred to add a little soap or other alkaline softening agent to the water in which the yarn is heated.

The process of the present invention is applicable to cellulosic textile materials of natural or

2

artificial origin; for example, the process may be applied to cotton or to artificial yarns of cellulose regenerated from viscose or cuprammonium cellulose solutions.

The following example illustrates the present invention, but the invention is not restricted to this example:

*Example*

Cakes of bleached, desulphurised 75 denier 18 filament viscose artificial silk are, without drying, placed in water in an autoclave and the temperature is raised to 120° centigrade. The treatment is continued for 15 minutes, the cakes are removed from the autoclave and dried. The yarn is wound from the cake on to bobbins and is then given a twist of 15 turns per inch. The twisted yarn is then steamed to set the twist. The steamed yarn is knitted into stockings which on subsequent dyeing give level shades.

20 What we claim is:

1. In the production of a dyed twisted cellulose yarn the combination with the steps of drying, twisting, setting the twist by a steaming operation and dyeing, of a preliminary step of treatment in water under pressure at a temperature above 100° centigrade to stabilise the dyeing affinity of the yarn against the effects of uneven steaming.

2. In the production of a dyed twisted cellulose yarn as claimed in claim 1 the addition of a small proportion of soap to the water used in the preliminary step.

3. In the production of a dyed twisted regenerated cellulose yarn the combination with the steps of drying, twisting, setting the twist by a steaming operation and dyeing, of a preliminary step of treatment in water under pressure at a temperature above 100° centigrade to stabilise the dyeing affinity of the yarn against the effects of uneven steaming.

4. In the production of a dyed twisted regenerated cellulose yarn as claimed in claim 3 the addition of a small proportion of soap to the water used in the preliminary step.

HORACE JAMES HEGAN.  
EDWIN HOLROYD SHARPLES.